

## UNITED STATES PATENT OFFICE

2,364,726

PROCESS FOR IMPROVING THE DYEINGS  
AND PRINTS PREPARED WITH WATER-  
SOLUBLE DYESTUFFS

Albert Landolt, Riehen, and Andreas Ruperti, Arlesheim, Switzerland, assignors, by mesne assignments, to the firm Ciba Products Corporation, Dover, Del.

No Drawing. Original application October 13, 1939, Serial No. 299,390. Divided and this application June 12, 1940, Serial No. 340,300. In Switzerland December 21, 1938

## 5 Claims. (Cl. 8—74)

This application is a division of our application for Letters Patent Ser. No. 299,390, filed October 13, 1939.

It is known that the wet-fastnesses of dyeings and prints, which have been prepared with the help of water-soluble dyestuffs, may be increased by aftertreatment with high-molecular organic compounds, if necessary in the form of their salts. As high-molecular compounds come inter alia in question those which are prepared by condensation of formaldehyde with compounds containing nitrogen. The latter may be capable or incapable of being hardened.

Among the high-molecular formaldehyde condensation products may be mentioned such as are derived from formaldehyde and nitrogen-containing compounds such as melamine, guanidine, guanyl urea, urea, dicyandiamide, etc. In this connection, compare U. S. patent specifications Nos. 2,093,651, 2,169,546 and 2,106,938.

Among the condensation products containing nitrogen, those are particularly valuable which are obtained by the condensation of formaldehyde with compounds which contain at least once the group



Such products are, for example, melamine, guanidine, guanyl urea, dicyandiamide, already mentioned.

This aftertreatment may consist of a simple wet treatment in baths which contain the products concerned. It may also consist of a wet treatment combined with a subsequent dry treatment at raised temperature, if formaldehyde-condensation products which are capable of being hardened are used as high-molecular organic basic compounds, whereby the fastness to wet treatment, in particular the fastness to washing, as a rule is still further improved. In both cases, however, the fastness to light may be unfavourably influenced.

It has now been found that this disadvantage may be eliminated if an aftertreatment with copper salts is combined with the aftertreatment with the aqueous solution of the high-molecular condensation products from formaldehyde and nitrogen-containing compounds. These combined treatments can be carried out one after the other in any desired order; it is however, preferable to unite them, so that the dyeings and the prints are treated at the same time with the organic and the copper compounds, for exam-

ple, with baths which contain copper salts in addition to salts of high-molecular organic basic compounds: if required, the dry treatment at raised temperatures may also hereupon take place.

As suitable copper salts, copper sulphate, copper nitrate, copper chloride, copper acetate, etc., may be mentioned.

## Example 1

10 A cotton or linen fabric is dyed on the jig with 3% Direct Sky Blue GS (Schultz, No. 510), rinsed and squeezed or hydro-extracted. The still moist material is padded on the mangle at room temperature through a solution containing per litre 15 30 gms. of a hydrophobic melamine-formaldehyde condensation product (obtained from 1 mol melamine and 6 mols formaldehyde), soluble in water in the ratio of 1:1, 20 10 ccm. formic acid 85% and 1 to 5 gms. copper chloride, or the equivalent quantity of another copper salt, such as copper formate or copper acetate. After drying, the fabric is subjected to a hardening treatment over heated cylinders for  $\frac{1}{2}$  minute at 130° C. The treated dyeing possesses very good fastness to light in addition to exceptional fastness to water and perspiration. By subsequent washing with soap and soda, the fastness to light is not decreased, so that here a permanent improvement in this property is concerned.

In place of Direct Sky Blue GS, many other dyestuffs may be used, giving the same result. 35 Among these may be mentioned Direct Blue RW (Schultz No. 507), Direct Brown M (Schultz No. 412), Chlorantine Fast Brown BRLL (Schultz vol. 2, page 48), Chlorantine Fast Violet 2RLL, Chlorantine Fast Yellow 4GLL, Chlorantine Fast 40 Orange T5RLL, Chlorantine Fast Grey 2BLL (all Schultz, supp. vol. 1, page 79).

## Example 2

A material composed of 70% wool and 30% 45 viscose-rayon staple fibre is dyed by known methods with 4% Chlorantine Brown BRLL (Schultz, supp. vol. 1, page 79) rinsed, hydro-extracted, and impregnated at room temperature with a solution containing per litre

50 30 parts by weight of a dicyandiamide-formaldehyde condensation product, obtained by condensation of 2 mols dicyandiamide with 3 mols commercial formaldehyde

15 parts by weight of formic acid 85% and

55 5 parts by weight of copper chloride,

after which it is dried without rinsing and hardened for 1 hour at 90° C. A dyeing possessing good fastness properties is obtained.

*Example 3*

A dyeing of Chlorantine Fast Orange TGLL on cotton material is impregnated with a solution containing per 100 parts water, 16 parts dimethylol-urea, 1 part ammonium phosphate, and 1 part copper chloride (the parts being by weight) and is then dried at 110° C., whereby the fastness of the dyeing to wet treatments is increased by the high-molecular compound formed. When the thus aftertreated dyeing is exposed to light, it exhibits a better fastness to light than a dyeing aftertreated in the same manner but with exclusion of the copper salt.

A similar result is obtained when Chlorantine Fast Orange TGLL is replaced by Chlorantine Fast Bordeaux B or by Chlorantine Fast Blue 3RLL.

What we claim is:

1. Improvement in the process of increasing the fastness properties of dyeings and prints, which have been obtained by means of a water-soluble dyestuff and aftertreatment with a high-molecular organic compound, produced by condensation of formaldehyde with a compound containing at least once the group



consisting in combining the aftertreatment with a simultaneous treatment with a solution of a copper compound in the same bath.

2. Improvement in the process of increasing the fastness properties of dyeings and prints, which have been obtained by means of a water-soluble dyestuff and aftertreatment with a high-molecular organic compound, produced by the condensation of formaldehyde with melamine, consisting in combining the aftertreatment with a simultaneous treatment with a solution of a copper compound in the same bath.

3. Improvement in the process of increasing the fastness properties of dyeings and prints, which have been obtained by means of a water-soluble dyestuff and aftertreatment with a high-molecular organic compound, produced by condensation of formaldehyde with a compound containing at least once the group



consisting in combining the aftertreatment with a simultaneous treatment with a solution of copper compound in the same bath, and then subjecting the material thus treated to a dry treatment at raised temperature.

4. Improvement in the process of increasing the fastness properties of dyeings and prints, which have been obtained by means of a water-soluble dyestuff and aftertreatment with a high-molecular organic compound, produced by the condensation of formaldehyde with melamine, consisting in combining the aftertreatment with a simultaneous treatment with a solution of a copper compound in the same bath, and then subjecting the material thus treated to a dry treatment at raised temperature.

5. A textile colored with a water-soluble dyestuff and aftertreated simultaneously with a high-molecular organic compound, produced by condensation of formaldehyde with a compound containing at least once the group



and with a solution of a copper compound, the wet-fastness of the aftertreated textile being superior and the light fastness thereof being of a magnitude at least equal to that of the untreated colored textile.

ALBERT LANDOLT.  
ANDREAS RUPERTI.